

# UNITED STATES PATENT OFFICE.

CARL HETTWIG, OF BERLIN, AND FRITZ HECKNER, OF BRAUNSCHWEIG,  
GERMANY.

## PROCESS OF PRODUCING ORNAMENTAL DESIGNS UPON WOOD.

SPECIFICATION forming part of Letters Patent No. 439,658, dated November 4, 1890.

Application filed February 21, 1890. Serial No. 341,361. (No specimens.)

*To all whom it may concern:*

Be it known that we, CARL HETTWIG and FRITZ HECKNER, subjects of the Emperor of the German Empire, residing, respectively, at Berlin and Braunschweig, in the German Empire, have invented certain new and useful Improvements in Process for Producing Ornamental Designs upon Wood, of which the following is a specification.

10 This our invention relates to a new process for tinging the natural surface of wood or producing thereon picturesque designs of different shades from a light-brown to a dark-brown color that will not fade from exposure to light 15 or to the changes of the weather. This process consists in the discovery of certain chemicals to be applied in successive order upon the natural surface of the wood and then the so-treated surface to be exposed to the chemical 20 action of the daylight.

It is a well-known process to coat the surface of metal, stone, or of a material of organic origin and of a homogene nature with a layer of varnish and then to tinge the open 25 spots or etchings with an acidiferous or coloring liquid for bringing forth a design upon the thus treated surfaces. For producing, however, an ornamental design upon the natural surface of wood has had its difficulties, caused 30 by the organic cellular construction of wood.

The varnishes for etchings are generally of a diaphanous and frequently of a coloring nature, and therefore must be removed after having served their purpose. For wood this 35 is not practical, because every mechanical operation of removal is liable to injure the surface of the wood, while a dissolving liquid in washing off the varnish is apt to soak into the wood and render its surface with an un-

40 clean appearance. It has been found necessary, therefore, to provide a varnish for coating the wooden surface around the spots to be tinged or colored that is colorless and transparent and will not require removal, but 45 contrary to remain as an advantageous protector and which will not produce a luster or burnish like the usual varnishes do. The varnish we have discovered to have the above- desired properties consists of a strong solu-

50 tion of caoutchouc in chloroform; and for the

purpose of preventing the solutions applied for bringing forth the design from spreading beyond the outlines of the design by running out into the fibers of the wood we previously soak the surfaces with a solution of alum in 55 the same manner as is usual for wood to be painted upon. After the surfaces of the wood have been thus treated with alum and the outlines of the design have been drawn or marked thereon in any usual manner, the 60 quickly-drying caoutchouc varnish is applied in proper conformity with the design upon all parts of the wooden surface not to be colored. Now the unvarnished surfaces of the wood are to be soaked with a solution of bi- 65 chromate of copper, (cuprum bichromicum,) and after this solution has been well absorbed, but before it has become dry, a solution of pyrogallic acid is applied. The so-treated wooden surface, still insignificantly showing 70 the design, is now exposed to the daylight, which slowly will bring forth a durable and chemically almost indestructible union between the bichromate of copper and the pyrogallic acid by chemical transformation under co-operation of the fibers of the wood, and within about twenty-four hours will be brought forth upon the tinged surfaces a more or less dark-brown color.

The two tinging solutions can be made and 80 applied in different proportions—that is, from one part of salt or acid in one hundred parts of distilled water up to the most concentrated solutions. With a stronger solution of bi- 85 chromate of copper and thereupon a weaker solution of pyrogallic acid we obtain greenish-playing color shades; and otherwise, again, a weaker solution of bichromate of copper combined with a stronger solution of pyrogallic acid will produce a reddish brown. Weak 90 solutions in general will produce a lighter coloring and stronger solutions darker colors, and thus in proportion as solutions of different strength are applied for different portions the design can be shaded, and thereby 95 wonderful effects can be produced. After the action of the daylight thereon the work is completed.

What we claim is—

1. The process of tinging the natural sur- 100

faces of wood for bringing forth thereon ornamental designs in different shades from a light-brown to a dark-brown color by first applying a solution of bichromate of copper, 5 next a solution of pyrogallic acid, and then exposing the so-treated surface to the daylight, substantially as set forth.

2. The process of producing ornamental designs of a brown color of different shades 10 upon wooden surfaces after the same have been soaked with a solution of alum, consisting of first coating the blank surfaces with a varnish consisting of a solution of caoutchouc

in chloroform, next for bringing forth the design in color the applying of a solution of bichromate of copper, and upon this again a solution of pyrogallic acid, and finally exposing the so-treated surfaces to the daylight, all substantially as set forth. 15

In testimony whereof we affix our signatures in presence of two witnesses. 20

CARL HETTWIG.  
FRITZ HECKNER.

Witnesses:

FREDK. V. S. CROSBY,  
ULRICH R. MAERZ.